# EUROPEAN PATENT APPLICATION

(11) **EP 1 460 137 A1**
(43) Date of publication of application: **22.09.2004**
(21) Application number: 04101109.9
(22) Date of filing: 18.03.2004
(51) Int. Cl.: C14C 9/02

(54) **Fatliquors and use thereof**

(30) Priority: 19.03.2003 IT VA20030011
(71) Applicant: Lamberti Spa, 21041 Albizzate (IT)
(72) Inventor: PERATELLO, Stefano Dr., 20045, Besana in Brianza (MI) (IT); ROALDI, Maria Grazia, 21015, Lonate Pozzolo (VA) (IT); GALANTE, Yves Dr., 20020, Arese (MI) (IT); LI BASSI, Giuseppe Dr., 21026, Gavirate (VA) (IT)

(57) **Abstract**

The present invention relates to leather fatliquors containing a protease, and to a fatliquoring method for tanned leather. The method of the invention is characterised by the use of a fatliquoring bath containing a protease and, in particular, a bacterial protease having its optimum of activity at alkaline pH.

## Description

This invention relates to leather fatliquors containing a protease, and to a fatliquoring method for tanned leather. The method of the invention is characterised by the use of a fatliquoring bath containing a protease and, in particular, a bacterial protease having its optimum of activity at alkaline pH.

The fatliquors of the invention confer to the product treated thereby excellent softness and resistance.

Fatliquoring is the step in the manufacturing of leather consisting in the application on tanned leather of fatty compounds which can be absorbed and improve its softness and elasticity; the application of such compounds normally takes place by immersing the leather in an aqueous dispersion of the fatliquors (the fatliquoring bath) and heat drumming.

With the term "fatliquor" we refer to the concentrated mixture of fatty compounds that in industrial application is dispersed into water to prepare the fatliquoring bath.

The fatliquors most commonly used in the manufacture of leather are natural oils, generally sulfonated or sulfitated, in the form of aqueous emulsion or dispersion; synthetic fatliquors are also known, such as high molecular weight esters of fatty acids with alcohols or polyols, mono- or di-sulfosuccinates of fatty alcohols, optionally ethoxylated and/or propoxylated, phosphoric esters of fatty acids, optionally ethoxylated and/or propoxylated and present in the form of salt.

In tannery, the use of enzymes (proteases and lipases) is widespread, but not in the fatliquoring step, nor the use of enzyme in this phase is described in the literature.

Enzymes are used in some acidic phases of the manufacture of hides or leather as tanning and re-tanning, at pH 2.5-5, and in the alkaline phase such as the beamhouse, at pH 7.5-13; enzymes are defined "acid" if they exhibit the maximum catalytic activity under acidic conditions, at pH 2.5-6, and "alkaline" if the maximum of activity is under alkaline conditions, at pH 7.5-12.

Normally, the pH value of the medium is of fundamental importance in the choice of the enzyme, and the enzyme shall have the maximum of catalytic activity around the pH value of the medium itself.

It has surprisingly been found that the use of a protease in the fatliquoring, and in particular of a bacterial alkaline protease, highly improves the breaking load, softness and elasticity of leather, while at same time favours the stable and uniform binding of the fatliquor.

The use of alkaline proteases in the fatliquoring bath is the more surprising as the fatliquoring step is carried out at acidic pH (from 5.5 to 7) and, in such pH conditions, alkaline proteases normally show a marked decrease of catalytic activity.

With the expression "alkaline protease" in the present text we refer to alkaline bacterial protease from *Bacillus subtilis,* natural of genetically modified.

It is an object of the present invention a fatliquoring method of tanned leathers characterised by the use of a fatliquoring bath containing from 0.01 to 10%, preferably from 0.1 to 5% by weight, of a protease, the percentage being referred to over the weight of the starting blue stockleather.

It is a further object of the invention the fatliquor for leather characterised by the fact that it contains from 0.01 to 5%, preferably from 0.5 to 2% by weight, of a protease.

According to a particularly advantageous aspect of the present invention, the protease is an alkaline protease.

The fatliquor of the invention contains from 30 to 80%, preferably from 50 to 70% by weight, of one or more active compounds selected in the group consisting of natural sulfonated or sulfitated oils, mono- or di-sulfosuccinates of fatty alcohols, optionally ethoxylated and/or propoxylated, high molecular weight esters of fatty acids with alcohols or polyalcohols, phosphoric esters of optionally ethoxylated and/or propoxylated fatty alcohols and present in the salt form.

For the realisation of the invention the preferred active compounds are those having ionic character, such as natural sulfonated or sulfitated oils, and mono- or di-sulfosuccinates of ethoxylated and/or propoxylated fatty alcohols; particularly preferred are mono- or di-sulfosuccinates of ethoxylated and/or propoxylated fatty alcohols having a number of mole of oxide higher than 7, described in the Italian patent application No. IT VA2001A000046.

The fatliquors of the invention are characterised by the fact that they are in the form of aqueous emulsion or dispersion.

It is well known and described in literature (for example in **KRAVETZ, L., et al** Effect of surfactant structure on stability of enzymes formulated into laundry liquids. *J Am Oil and Chem Soc* 1985, vol. 62, no. 5, p. 943-949. and in **STAUFFER, C.E., et al** *. Biochimica et Biophysica Acta,* 1973, vol. 295, p. 457-466. ) that aqueous formulations containing enzymes and substances having anionic character are not stable over time: enzymes, more noticeably proteases, are rapidly and irreversibly denatured and deactivated by the presence of such substances so that their catalytic activity is lost.

Surprisingly, the faliquors of the invention are stable and maintain their properties unchanged over time.

The faliquors according to the invention are stable for at least two months at temperature of 0-35°C.

For the realisation of the present invention the fatliquoring step is conducted, with the usual procedure, in a fatliquoring bath containing from 3 to 20%, preferably from 5 to 15% by weight, of one or more active substances selected from the group consisting of natural sulfonated or sulfitated oils, mono- or di-sulfosuccinates of fatty alcohols, optionally ethoxylated and/or propoxylated, high molecular weight esters of fatty acids with alcohols or polyalcohols, phosphoric esters of optionally ethoxylated and/or propoxylated fatty alcohols and present in the form of salt, the percentage being referred to the weight of the starting blue stock.

The fatliquors of the present invention are particularly suitable for leather clothing and gloves and for furniture and car upholstery.

The resulting leather is softer and more resistant than the one obtained with the analogous fatliquor lacking in protease.

Another characteristic that makes the use of the fatliquors of the invention especially attractive is the fact that with an equal amount of active substances in the fatliquoring bath, the active substances themselves are better fixed, absorbed in higher quantity and more uniformly distributed, as illustrated by the following examples.

### Example 1 (comparative).

An entire wet blue cowhide is longitudinally cut in two pieces (Wet Blue A and Wet Blue B).

Wet Blue A is treated as described hereafter.

All percentages are by weight and based on the starting blue stock.

The wet blue is given a thirty minute water wash, at 35 °C with 200% of water and 0.5% of Alkilarol NF (an anionic surfactant commercialised by Lamberti S.p.A.).

The drum is drained.

150% water, 1 % of sodium formate, 0.2% of sodium bicarbonate are added and the mixture is then drummed (mixed) for 30 minutes at 35 °C. The pH of the bath is 4.5.

4% of Reotan PM (acrylic resin commercialised by Lamberti S.p.A.) and 0.5% of Lamtan TN Liq. (synthetic tannin commercialised by Lamberti S.p.A.) are then added and the mixture is drummed (mixed) for 30 minutes. 4% of Lamtan CRT (synthetic tannin commercialised by Lamberti S.p.A.) is then added to the drum and the mixture is drummed (mixed) for 60 minutes.

The drum is left in automatic rotation during the night.

The drum is then drained, the stock is washed and then a new bath is prepared with
200% water at 35 °C;
2% of sodium formate
2% of sodium bicarbonate.

The mixture is drummed (mixed) for 90 minutes.

The drum is then drained.

For the fatliquoring step, 200% of water and 12% of a fatliquor consisting of
- 65 parts by weight of sulfosuccinic monoester of 30 moles propoxylated and 3 moles ethoxylated cetyl stearyl alcohol
- 35 parts by weight of water
are added and the mixture is drummed for 60 minutes.

1 % of formic acid is then added and the mixture is drummed (mixed) for 20 minutes.

The drum is then drained.
150% of water at 35 °C and 0.5% of Alkilarol NF are then added and
the mixture is drummed (mixed) for 20 minutes.

The drum is then drained and the leather is dried at ambient temperature for 24 hours (Leather A)

### Example 2.

Wet Blue B is treated as described for Wet Blue A in Example 1, but using in the fatliquoring step a fatliquor consisting of:
- 65 parts by weight of sulfosuccinic monoester of 30 moles propoxylated and 3 moles ethoxylated cetyl stearyl alcohol
- 34 parts by weight of water
- 1 part by weight of Purafect 4000 L (bacterial protease from Bacillus subtilis commercialised by Genencor Int.)

The leather is dried at ambient temperature for 24 hours (Leather B)

Evaluation tests for Leather A and Leather B.

Leather A and Leather B, obtained from Example 1 and 2, are evaluated by the following methods
1. Softness: 10 persons are asked to evaluate tactually which is the softer leather; 10 out of 10 repute Leather B softer than Leather A (comparative leather).
2. Amount of absorbed fatliquor: the amount is determined by a COD measure. The CODs (Chemical Oxygen Demand) of the two exhausted fatliquoring baths from Example 1 and Example 2 (Bath 1 and Bath 2) are measured by Kit LANGE LCK 114 (DIN 38409-H-41). A low COD value corresponds to a better absorbency of the fatliquor onto the leather. The results are reported in Table 1.
3. Amount of absorbed fatliquor: the amount is also determined by extracting from the leather the fatty substances, according to method IUC No. 4 (IUC standard test methods are emitted by the International Union of Leather Technologists and Chemists Societies). The results (grams of fatty substances extracted from 100 grams of leather) are reported in Table 2 and show that Leather B has absorbed a higher amount of active substances from the fatliquor.

**Table 1**

| | COD (mg O₂/l) |
|---|---|
| Bath A | 8.340 |
| Bath B | 6.600 |

**Table 2**

| | g/100g |
|---|---|
| Leather A | 10 |
| Leather B | 12.5 |

### Example 3 (comparative).

A blue wet cowhide is treated as described in Example 1 (Leather C)

### Example 4

A blue wet cowhide is treated as described in Example 2 (Leather D)

### Evaluation tests for Leather C and Leather D.

Evaluation of the persisting of enzymatic activity in the fatliquoring step by means of the fogging test.

The fogging of Leather C and D and the fogging of two pieces of the same leather treated as described in Example 1 but not subjected to fatliquoring (Leather C' and Leather D') are measured according to standard DIN 75201, both by the gravimetic test and by the reflectance test.

The leathers having the better fogging characteristics are those showing lower values from the gravimetric test and higher values from the reflectance test. The results are reported in Table 3. It is be observed that Leather C improves its fogging characteristics in respect of Leather C', while Leather D worsens its fogging characteristics in respect of leather D'.

The worsening of the fogging characteristics is due to the increase of the overall released substances, which are in part generated by the proteolysis of the collagen fibres; the worsening of these characteristics in Leather D is therefore also an indication of the fact that the protease present in the fatliquoring bath maintained its catalytic activity.

**Table 3**

| | Reflectance fogging test (%) | Gravimetric fogging test (g/50 cm²) |
|---|---|---|
| Leather C' | 88.02 | 1.70 |
| Leather C | 91.60 | 1.20 |
| Leather D' | 98.67 | 0.75 |
| Leather D | 94.05 | 3.65 |

### Example 5 (comparative).

An entire wet blue ovine hide is longitudinally cut in two pieces (Wet Blue OVA and Wet Blue OVB).

Wet Blue OVA is treated as described in Example 1 (Leather OVA).

### Example 6.

Wet Blue OVB is treated as described in Example 2 (Leather OVB).

### Evaluation tests for Leather OVA and Leather OVB.

Resistance: Leather AVA and Leather OVB are evaluated determining the breaking load with standard test method IUP 36 (IUP standard test methods are emitted by the International Union of Leather Technologists and Chemists Societies). The results are reported in Table 4 and show that Leather OVB is more resistant than Leather OVA.

**Table 4**

| | Breaking Load (Kg/mm²) |
|---|---|
| Leather OVA | 12.28 |
| Leather OVB | 19.60 |

## Claims

1. Leather fatliquor **characterised by** the fact that it contains from 0.01 to 5.0% by weight of a protease.

2. Leather fatliquor according to claim 1., **characterised by** the fact that it contains from 0.5 to 2.0% by weight of a protease.

3. Leather fatliquor according to claim 1. or 2., wherein the protease is an alkaline protease.

4. Leather fatliquor according to anyone of the preceding claims, containing from 30 to 80% by weight of one or more active substances selected from the group consisting of natural sulfonated or sulfitated oils, mono- or di-sulfosuccinates of fatty alcohols, optionally ethoxylated and/or propoxylated, high molecular weight esters of fatty acids with alcohols or polyalcohols, phosphoric esters of optionally ethoxylated and/or propoxylated fatty alcohols and present in the salt form.

5. Leather fatliquor according to claim 4., containing from 50 to 70% by weight of one or more active substances.

6. Leather fatliquor according to claim 5. or 6., wherein the active substances are selected from the group consisting of natural sulfonated or sulfitated oils, and mono- or di-sulfosuccinates of ethoxylated and/or propoxylated fatty alcohols.

7. Leather fatliquor according to anyone of claims from 4. to 6., wherein the mono- or di-sulfosuccinates of ethoxylated and/or propoxylated fatty alcohols have a number of mole of oxide higher than 7.

8. Leather fatliquor according to anyone of the preceding claims in the form of aqueous emulsion or dispersion.

9. Method for the fatliquoring of leather **characterised by** the use of a fatliquoring bath containing from 0.01 to 10% by weight of a protease.

10. Method for the fatliquoring of leather according to claim 9., wherein the fatliquoring bath contains from 0.1 to 5% by weight of a protease.

11. Method for the fatliquoring of leather according to claim 9. or 10. wherein the protease is an alkaline protease.

12. Method for the fatliquoring of leather according to anyone of the claims from 9. to 11., wherein the fatliquoring bath contains from 3 to 20% by weight of one or more active substances selected from the group consisting of natural sulfonated or sulfitated oils, mono- or di-sulfosuccinates of fatty alcohols, optionally ethoxylated and/or propoxylated, high molecular weight esters of fatty acids with alcohols or polyalcohols, phosphoric esters of optionally ethoxylated and/or propoxylated fatty alcohols and present in the salt form, the percentage being referred to over the weight of the starting blue stockleather.

13. Method for the fatliquoring of leather according to claim 12., wherein the fatliquoring bath contains from 5 to 15% by weight of one or more active substances, the percentage being referred to over the weight of the starting blue stockleather.

14. Method for the fatliquoring of leather according to claim 12. or 13., wherein the active substances are selected from the group consisting of natural sulfonated or sulfitated oils, and mono- or di-sulfosuccinates of ethoxylated and/or propoxylated fatty alcohols.

15. Method for the fatliquoring of leather according to claim 14., wherein the mono- or di-sulfosuccinates of ethoxylated and/or propoxylated fatty alcohols have a number of mole of oxide higher than 7.
